

Oct. 14, 1924.

1,511,637

G. SPACKELER ET AL

METHOD FOR THE DRESSING OF MINERAL CONGLOMERATES OR MIXTURES

Filed Aug. 4, 1923

Fig. 1



Fig. 2



Fig. 3



Fig. 4



Fig. 5



Fig. 6



Fig. 7



INVENTORS

Georg Spackeler  
Karl Ginz  
By Richards, Sculley & Sons

## UNITED STATES PATENT OFFICE.

GEORG SPACKELER, OF CLAUSTHAL, AND KARL GLINZ, OF BERLIN-DAHLEN,  
GERMANY.

## METHOD FOR THE DRESSING OF MINERAL CONGLOMERATES OR MIXTURES.

Application filed August 4, 1923. Serial No. 655,767.

*To all whom it may concern:*

Be it known that I, GEORG SPACKELER, a citizen of Germany, residing at Clausthal, Germany, and I, KARL GLINZ, a citizen of 5 Germany, residing at Berlin-Dahlem, Germany, have invented certain new and useful improvements in a Method for the Dressing of Mineral Conglomerates or Mixtures, of which the following is a specification.

This invention relates to a process for the dressing of ores and other grown mineral conglomerates. According to the commonly used dressing of ores and similar grown 15 mineral conglomerates the blocks of ore are crushed, previously to the dressing, in a crushing machine, for instance in a stone breaker, crushing mill or ball mill to a determined size of grain, whereupon the dressing 20 is effected by means of settling processes or the like, and the average products thus obtained are further crushed. This treatment does not take into consideration the natural condition of the ores or 25 conglomerates as the ore is broken indiscriminately so that each grain of the crushed product contains substantial proportions of all of the different constituents of the ore. In this manner average products are obtained 30 which have to be subsequently treated wherefrom results a more extensive crushing of the ores and a more considerable undesirable formation of slime than would be necessary according to the natural condition 35 of the ore.

This invention has for its object to avoid as much as possible an unnecessarily extensive crushing of the ore and conglomerates in dressing and to utilize the natural separation joints in the ore to facilitate the dressing process.

The improved method is especially adapted for ores which have been produced by the depositing of different mineral constituents 45 individual mineral grains consisting substantially wholly of homogenous masses of the respective constituents, homogenous substances being for instance cemented by a binding matter. As examples of such ore oolitic ore or so-called bean ore may be cited. With such ores, even if they break in solid lumps, fine fissures exist between the 50 surfaces of the different individual mineral bodies homogenous per se and between these and the binder, said fissures being filled with

air, or the binding matter itself consists of conglomerates permeable to air, for instance sand-like conglomerates.

The method according to this invention has for its object to destroy artificially, by 60 a convenient treatment, the cohesion in these fissures or to enlarge these fissures so that the mineral conglomerate falls to pieces automatically or may be cleaved by mechanical means with the expenditure of little energy. 65

According to the invention, the material to be dressed is submitted in a closed chamber to the action of vacuum in order to evacuate the air. At the same time or later on water is made to flow into the fissures to replace 70 the air, or water is forced into the fissures by fluid pressure. The vacuum and the pressure may be applied constantly or alternately. The hydraulic pressure may for instance vary between zero and minus, or between zero and plus or between plus and minus. The disintegration of the material may be facilitated by simultaneous shaking or knocking movements.

This method is especially adapted for the 80 treatment of ore in which smooth separation surfaces exist between the several constituents, for instance iron ore found in many sedimentary deposits in Germany and other countries. These ores consist of granular 85 pieces generally cemented by a binding matter which is mostly calcareous or siliceous.

The usual dressing of these ores presents the difficulty that, when crushing machines are used, the ore nodules are completely 90 crushed so that great quantities of the ore disintegrate in the shape of a slime which can be scarcely utilized, nodules of marl and fine grained ore particles also being formed notwithstanding a great consumption

95 of water, which nodules impede the dressing, as they are almost in crushable owing to their viscosity and as on the other hand they cannot be dissolved in water. The formation of such nodules is avoided 100 according to this invention, the ore being at the same time crushed easily to form a product which contains almost all iron nodules and beans as single pieces free from admixtures. In experiments made with the 105 iron ore which had been disintegrated and separated according to this invention an essentially greater quantity of ore in lumps was obtained in the jigger and in the spitzkasten with subsequent classifying, viz., 110

in the normal dressing process, than without the improved method. In one single dressing operation concentrations of the very poor ores, which as crude ores contained only 22-23% Fe were obtained up to 40-44% Fe in the concentrate and the silicic anhydride ( $SiO_2$ ) of which in the crude ore 25-30% were contained, was reduced to 10-12%. The coarser kinds of ore amounted to  $\frac{3}{4}$  of the whole concentrate, all ores over 1 mm. size of grain being called coarser ores. Also in the ores of less than 1 mm. size of grain an essential reduction of the silicic anhydride and a concentration up to 40% iron was possible. In all the experiments which have been formerly made with these ores such results as obtained according to the improved method have never been obtained.

20 The treatment for loosening the bonds may be continued until the conglomerate disintegrates into its constituents.

With other conglomerates of this kind which do not disintegrate readily this treatment is followed by a mechanical treatment for cleaving the material in accordance with its natural depositing surfaces.

30 A further object of the invention is to exert upon the material in mass a kneading pressure in order to further loosen the bonds until the different constituents of the conglomerate are mutually shifted. The result is that the lumps of ore are not accidentally broken but are separated along the natural 35 surfaces of separation. As these surfaces of separation are mostly identical with the limiting surfaces of the different mineral constituents, the several mineral grains of approximately homogenous character remain undivided, the conglomerate being disintegrated into its constituents. By the crushing process an almost complete dressing is therefore obtained at the greatest possible size of the grains, so that the subsequent concentration is considerably simplified.

40 This step of the improved method may be executed in various manners; a tightly packed heap of material, the structure of which has been loosened, may for instance be submitted in a closed or semi-closed chamber under moderate pressure by a plunger to a kneading treatment.

50 It is evidently advisable to work also in this case continuously. With this object in view the working chamber may have the shape of a launder in which the plunger works. The inlet and outlet are open and the advance of the material in mass is produced by the fall or by a water current or by both.

60 This manner of crushing may be made the basis of a continuous dressing method, a concentration process known per se following directly on the disintegration of the

mineral mixture which has been previously loosened. The water designed to make the material advance may be preferably used for this purpose, its flow being regulated in such a manner that the material is sized according to the specific weight. A classifying device of known type may further be connected with the launder which conveys the disintegrated material, whereby the grains of different sizes of the material are separated for instance by means of grading sieves. The remaining pulp contains in suspension valuable particles of the mixture together with worthless ones, which possess little tendency to precipitate. The pulp may therefore be worked up by differentiating separation of the suspended particles by means of flotation or with the aid of chemical reagents.

Several forms of construction of the apparatus designed for the application of the improved method are shown by way of example in the accompanying drawing, wherein:

Figs. 1 and 2 show two species of apparatus with closed pressure chamber for intermittent working.

Figs. 3 and 4 show a launder shaped chamber for continuous working in plan view and in section on line A-B of Fig. 3

95

respectively.

Figs. 5 and 6 show a similar form of construction as Figs. 3 and 4 respectively in

100

plan view and in section on line C-D of Fig. 5.

Fig. 7 shows a fourth form of construction in plan view.

In the form of construction shown in Figs. 1 and 2 a quantity *a* of the loosened conglomerate is charged into a cylinder *b* in which it is submitted to moderate pressure from two sides by plungers *c*. By the heaping of the material the breaking

105

of the several constituents is avoided; the constituents shift on one another along the natural fissures between the layers so that

110

they are separated from one another without application of considerable energy. The pressure of the plungers may be constantly progressing or intermittent or alternating.

115

In the form of construction shown in Fig. 2 the cylinder *b* is closed at the lower end and the kneading is effected by one single plunger *c*.

120

According to Figs. 3 and 4 a launder *d* open at both ends is used together with a plunger *c* working in the same. The walls of the launder as well as of the plunger are preferably sloping to the lower end in order

125

to increase the action of mutually shifting and kneading the different constituents of the mixture. The material in bulk is admitted at one end of the launder under the plunger and it is conducted towards the outlet end by the fall in the launder or by

130

the action of a water current while being continuously submitted to a kneading treatment by the plunger.

In the form of construction shown in Figs. 5 and 6 the arrangement is similar, but the plunger leaves the launder partly open at the upper end. The kneading effect is not impaired as by the mutual friction the particles are prevented from giving way.

In the form of construction shown in Fig. 7 the launder as well as the plunger are of zig-zag-shape. The cross section is the same as in Fig. 4.

15. What we claim is:

1. The process of preparing conglomerate ore for recovery of valuable constituents thereof, consisting in subjecting the same intermittently to vacuum until the bonds 20 between granules thereof are loosened.

2. The process of preparing a conglomerate ore for recovery of valuable constituents thereof, consisting in subjecting the same intermittently to vacuum until the bonds 25 between granules thereof are loosened, and subjecting the material so treated to mechanical agitation to complete disintegration of the mass.

3. The process of preparing a conglomerate ore for recovery of valuable constituents thereof, consisting in subjecting the same intermittently to vacuum until the

bonds between granules thereof are loosened, subjecting the material so treated to mechanical agitation to complete disintegration of the mass, and adding liquid to the mass to promote disintegration. 35

4. The process of preparing conglomerate ore for recovery of valuable constituents thereof, consisting in subjecting the same 40 alternately to vacuum and to superatmospheric pressure until the bonds between the granules thereof are loosened.

5. The process of preparing conglomerate ore for recovery of valuable constituents 45 thereof, consisting in subjecting the same alternately to vacuum and to superatmospheric pressure until the bonds between the granules thereof are loosened, and subjecting the material so treated to mechanical 50 agitation to complete disintegration of the mass.

6. The process of preparing conglomerate ore for recovery of valuable constituents thereof, consisting in subjecting the same 55 alternately to vacuum and to superatmospheric pressure until the bonds between the granules thereof are loosened, and adding liquid to the mass to promote disintegration.

In testimony whereof we have affixed our 60 signatures.

GEORG SPACKELER.  
KARL GLINZ.